

May 23, 1939.

H. W. GREIDER ET AL

2,159,586

BITUMINIZED WEB

Original Filed July 20, 1933

*Fig. 1.*



*Fig. 2.*



INVENTOR  
Harold W. Greider  
George Arthur Facold  
BY  
George H. Mills, Jr.  
ATTORNEYS

## UNITED STATES PATENT OFFICE

2,159,586

## BITUMINIZED WEB

Harold W. Greider, Wyoming, and George Arthur Fasold, Cincinnati, Ohio, assignors to The Philip Carey Manufacturing Company, a corporation of Ohio

Original application July 20, 1933, Serial No. 681,286. Divided and this application May 26, 1937, Serial No. 144,984

4 Claims. (Cl. 91—68)

This case is a division of application Ser. No. 681,286, filed July 20, 1933, (Patent No. 2,105,531 issued Jan. 18, 1938) which is incorporated herein as a part of the disclosure of the present invention. The apparatus, method and article are all disclosed in the parent case, but the subject thereof is the method.

This invention relates to waterproofed web material, and particularly pertains to woven or 10 felted web material, such as felt, paper fabrics and the like impregnated with and/or coated with bituminous composition to be used as building material and the like for weather resisting covering such as roofing, siding and the like.

15 Two serious defects encountered in bituminized fabric roofing as heretofore made, have been its tendency to "blister" and "slide", and it is the aim of this invention to provide waterproofing web material for the manufacture of bituminized roofing having neither of these objections.

20 Bituminized building material heretofore employed for roofing and siding contained a considerable number of voids caused by incomplete saturation with asphalt and entrapment of air 25 during its manufacture. Accordingly when the material is exposed to the weather, moisture is absorbed either by direct application of water or by contact with moist air. This is due chiefly to the porosity of the sheet that results from 30 incomplete saturation and entrapment of air, but also in part to the porosity of the pulverulent or granular material which is adhered thereto and apparently affords communication with the internal minute air pockets or voids either through 35 or along the sides of the granular particles. Tests have shown that many roofing felts and roofings heretofore made when soaked in water for one hour at 120° F. will absorb as much as 10% to 20% of water or will absorb from 10% to 40% water in twenty-four hours at 77° F. Further tests have shown that when such porous moisture-laden roofing is exposed to hot summer weather, a multiplicity of bubbles or blisters about  $\frac{1}{8}$  inch to about  $\frac{3}{4}$  inch in diameter are formed 45 which push up to the surface of the roofing, eventually burst open and thus expose the felt base to the weather. The felt being unprotected at the blister points deteriorates rapidly. Moreover, a blistered roofing, particularly when the 50 blisters are broken, is very unsightly as well as of low resistance to weathering.

55 Sliding results from the tendency of the bituminous surface coating and the adhered granular weather resisting material to move or slip with respect to the fabric foundation or base

when exposed to summer heat. Sliding, of course, is particularly serious on inclined roofs or vertical walls. Frequently shingles of ordinary size exhibit  $\frac{3}{4}$  inch or more slide after having been in place for some time. Sliding, of course, is 5 ruinous both to the appearance and the weather durability of the roofing.

It is the aim of this invention to provide a roofing material which is devoided of air and effectively sealed against the penetration of air 10 and moisture, and has included in its structure a layer which is of a character and is so associated with the foundation as to prevent relative movement of the components making up the roofing material. In other words, the aim of the 15 invention is a roofing material which is substantially non-blistering and/or non-sliding. More specifically one of the features of the new roofing is that it is substantially completely devoided of air and contains a layer of web material 20 impregnated with a bituminous saturant and second layer of web material impregnated with bituminous material having a substantially higher softening point than said saturant. In a preferred embodiment of this invention the air-devoided roofing contains an inner layer of web material and two layers of web material which 25 are on each side of said inner layer and which are impregnated with a bituminous material having a substantially higher softening point than 30 the softening point of the saturant for the inner layer. Further features of this invention reside in the fact that the webs of the layers are felts and that the felts of these layers are inter-felted. Thus, a felt is impregnated with a 35 saturant of one softening point and also impregnated adjacent the surface or surfaces thereof with a bituminous material of substantially higher softening point, the bituminous material of higher softening point sealing the air-devoided 40 felt and being keyed to the felt. A further feature resides in the combination with a bituminized web impregnated with a bituminous saturant and also impregnated within its surface layer or layers with a bituminous material having a higher softening point than the saturant, of a bituminous coating which is integrally bonded with the higher softening point bitumen and which has a higher softening point than the saturant. Thus the product not only contains 45 coating material of relatively high softening point impregnated in a surface layer of the felt and keyed thereto but also a second layer of higher softening point bituminous coating material 50 contacting with the higher softening point bitu-

20

25

30

35

40

45

50

55

minous material impregnated in the felt. This structure affords great resistance to sliding because there is no low softening point bitumen at the surface to act at high roof temperatures as a lubricant between the felt and the coating bitumen and because the coating bitumen is keyed to the felt. It affords great resistance to blistering because the high softening point bitumen used as the surface sealing layer is applied while the impregnated sheet is devoided of and unexposed to air.

It is a further feature of one embodiment of this invention that there is employed in combination with a web impregnated with a saturant and sealed with a coating material having a higher softening point than said saturant, a second coating material which has a higher softening point than the saturant and which contains a mineral filler.

A further feature of roofing embodying this invention is that the coating material which does not impregnate the web but overlies the same can be of reduced thickness and weight. Thus, when the web is completely impregnated and all its voids filled with bituminous saturant and part of the coating bitumen is impregnated in the surface of the web, less coating has to be used overlying the web to attain a desired finished weight of the roofing and this fact coupled with the keying of the coating to the web and the contacting of coating impregnated in the web with coating overlying the web, results in a finished product which is very resistant to sliding.

In the new roofing of this invention the web of felt, for example, is protected perfectly. It is completely impregnated with a bituminous saturant and it is sealed in a devoided condition so that it is substantially non-porous and so prevents moisture from entering and causing blistering and deterioration of the web. The saturant, sealing layer and coating layer become virtually a single, integral, non-porous waterproofing layer; hence the roofing embodying this invention has a greater durability and resistance to weathering. This is true whether weathering action is applied to the roofing on the weathering surface or at cut edges. Roofing heretofore made has been particularly susceptible to penetration of moisture from cut edges with particularly rapid deterioration at such points. In the new roofing of this invention the portion exposed by cut edges is substantially free of voids and moisture is unable to penetrate and to cause deterioration.

It is a further feature of the new product of this invention that the water absorption is very low. Thus samples of roofing material to be substantially non-blistering should have less than 2.0% water absorption when soaked in water for 24 hours at 77° F. and a product having less than 2.0% of water absorption under the above conditions is to be regarded as coming within the scope of this feature of this invention. By the practice of this invention it has, in fact, been found possible to produce roofing having less than 0.5% void, as determined by soaking the roofing in water at 77° F. for 24 hours.

Further purposes, features and advantages of this invention will become apparent in the following description of the illustrative embodiment of this invention in connection with the accompanying drawing, wherein:

Fig. 1 is a sectional view of a roofing material embodying the invention; and

Fig. 2 is a sectional view of a modified form of roofing embodying the invention.

Referring to the drawing in which like numerals are used to designate like parts, a web 78 of suitable fibrous material, preferably felt, is impregnated with a saturating material 79. One method of saturating is to unroll the web from a supply roll or rolls and pass it progressively through a saturating tank containing the saturating material heated from about 350° F. to 400° F., although the temperatures named are not regarded as critical.

The saturating material 79 is preferably a relatively low softening point asphalt. The lower softening point asphalts undergo deteriorative oxidation and hardening less rapidly on weathering and are more flexible. Moreover, in melting them sufficiently to make them fluid enough to permit a web to be impregnated therewith, they do not have to be heated to temperatures which are so high that burning and weakening of the web occurs during the time that is required to impregnate a dry web. Preferably, a saturant is used which has a softening point of about 95° F. to 140° F. as determined by the ball and ring method and which has a penetration of about 10 to 130 at 77° F. as determined by the Dow penetrometer. Considerable latitude below and above the preferred ranges above given, e. g., the use of materials having a softening point of about 75° F. to about 200° F. with a penetration of about 5 to 200 at 77° F. is permissible, having in mind that if a bituminous saturant having too low a softening point is used, the product will be too soft and too flexible and that if a saturating material having too high softening point is used there is likelihood of burning the web during the saturating step and of producing a product which is too rigid and subject to excessive cracking when flexed and of reduced resistance to weathering.

During the immersion of the web in the bath of bituminous saturant, it may be advantageously passed alternately over any number of rolls disposed in the saturating tank to be submerged below the surface of the saturant, thereby causing thorough impregnation of the web with the saturant. Excess saturant is removed from the web after it emerges from the saturant bath. It has been found in practice that it is desirable to have sufficient excess saturant removed to leave the web in a "spotted" condition, namely, having certain areas appearing wet and certain areas appearing dry. If too great amounts of saturating material are left adhering to the surface of the web, this material acts as a lubricant for higher melting point coating applied thereto with the result that the finished product has a tendency to slide. If the saturated felt is made too "dry", it is difficult to remove all the air from the felt prior to the coating and sealing of the felt.

The saturated web is then treated with bituminous sealing material 80 prepared with a harder consistency and of a higher fusing point than the saturant. It has a softening point preferably between about 220° F. and about 250° F. and a penetration of about 9 to 20 at 77° F. However, satisfactory results can be obtained when the softening point ranges from about 190° F. to about 275° F. and the penetration ranges from about 50 to 5 at 77° F. The sealing material is preferably applied at about 425° F. although about 50° to 75° F. variation from this range will still afford satisfactory results.

The sealing material 80 is applied while the saturated web is substantially devoided of air, and this may advantageously be carried out by

progressively passing the saturated web through another tank containing the sealing material 80 heated to a fluid condition. Squeezing means, such as a pair of squeeze rolls, may be disposed 5 in the tank, submerged below the surface of the molten sealing material, to expel air from the saturated web. The sealing material is applied while the saturated sheet is voided of air and while compressed. Accordingly re-entry of air 10 is precluded by the sealing means, and as the saturated web tends to re-expand, upon release of the compressing force, the sealing material is drawn into the voids from which the air has been expelled, thereby sealing the saturated web 15 against the entry of air and providing in the surface thereof a layer filling the surface interstices to a substantial depth and interlocking with the web. An excess amount of sealing material may be applied to the web in order to provide a coating layer of the sealing material on the surface of the saturated web as well as impregnated therewith, or any excess may be removed leaving only a sealing layer impregnated 20 to a substantial depth beneath the surface of the web.

25 It is preferable in the practicing of the invention that the sealing material be applied as quickly as possible after the saturating so as to avoid the absorption of air by the web which would otherwise occur due to the cooling of the web and expansion thereof after having passed the compressing means. Preferably, although it is not essential to the practice of the invention, the web is not permitted to cool substantially, e. g., more 30 than a few degrees, in passing from the saturating bath to the coating bath. Immersion of the web in the hot sealing material partially voids it, and while immersed in the bath of sealing material, it is compressed preferably to a defi- 35 nitely greater extent than that resulting from the use of any doctor means for removing the excess saturant at the conclusion of the saturating bath. After compression is released, the web, covered with the sealing material, expands 40 and draws in said sealing material to replace the air that has been expelled. Accordingly, the web is thus not only filled with saturant but also is sealed with the sealing material which permeates 45 the web surface and keeps the web in a permanently voided condition. It is to be noted that the web is maintained voided during application of the sealing material. After the web has 50 been filled with the saturant and sealed with the sealing material as above described, it may be used without further treatment, other than being subdivided into smaller units, cut from the sheet. It is adapted for various uses such as 55 flooring, built-up roofing, pipe line covering and the like.

60 For roofing purposes, however, it is preferable to apply a coating layer 82 of the same character and composition as the sealing material to give increased thickness, resistance to weathering and to afford a layer of sufficient thickness to hold 65 adherently a finely divided, e. g., granular solid material 83, such as slate granules of suitable color. It is preferable to apply this coating before cooling the sealed web. Additional coating with bituminous material can be applied if desired but 70 ordinarily is not necessary. The underside or non-weather side of the web can be coated with pulverulent material 81 such as fine mica flakes. In this structure, there is an inner portion of 75 felt impregnated with an inner layer of saturant

ed with outer layers of sealing material having a higher softening point than said saturant. The bituminous material in layers 80 and 82 are substantially identical and become merged with one another so that a coating is afforded comprising 5 bituminous material which impregnates the felt and is keyed thereto and a surface layer 82 which overlies the felt and which has substantial thickness and weather-resistance.

A modified embodiment of the invention is 10 shown in Fig. 2. The structure in Fig. 2 is identical with that of Fig. 1 except that in place of the layer 82 shown in Fig. 1 a layer 84 is employed of coating material which is substantially different from the coating material contained in 15 layer 80. Thus, for example, a coating material having a different softening point from the melting point of the coating material contained in layer 80 may be employed. Moreover, the coating material in layer 84 may comprise a bituminous 20 layer having dispersed therein a finely divided inorganic solid material in certain cases as desired.

It is preferable that the roofing contain less than about 2.0% of voids. Moreover, it is also 25 preferable that the total weight of material overlying the felt base of the roofing and including the bituminous coating material and finely divided solid surfacing material be less than about 45 pounds per 100 sq. ft. so as to minimize a tendency 30 of overlying material to slide.

The new product of this invention may also be manufactured without layer 82 or layer 83, for example, to be used as the felt in built-up roofing construction. Moreover, a variety of superficial coatings of dust or granular materials, or liquids such as paint and the like, may be applied for protective or ornamental purposes, or 35 both.

While the invention has been described in connection with certain specific illustrations, it is to be understood that this has been done for the purpose of illustration and that the invention is not to be limited thereby. Moreover, it is also to be understood that the term "roofing" includes 40 roll and shingle roofing, siding strips, and other building materials of the character described.

We claim:

1. As a roofing material, a compressible fibrous substantially completely filled and sealed web 50 material impregnated with a bituminous saturant and squeezed by pressure, mechanically applied to the surfaces on the opposite sides thereof, to a substantially voided condition and sealed on the opposite sides thereof in said substantially de- 55 voided condition with a sealing layer of bituminous sealing material applied to said surfaces of said mechanically squeezed web which bituminous sealing material has a higher softening point than the softening point of said saturant 60 and which bituminous sealing material is integrally bonded with said saturant and with the fibers of said web adjacent to and at said surfaces of said squeezed web and fills the surface interstices of said web to substantial depth with 65 avoidance of substantial porosity, the remainder of said web material being so completely filled with said saturant as to be substantially free of voids, thereby affording a bituminized web which is substantially completely filled and sealed so 70 as to be highly resistant to blistering.

2. A roofing material according to claim 1, which has overlying at least one surface of said felt an outer layer of bituminous sealing material having a softening point substantially high- 75

er than the softening point of the saturant and has a finely-divided solid material adhering to said outer layer, the total weight of material above said surface of said felt being less than 45 pounds per 100 sq. ft.

3. As a roofing material, a compressible fibrous filled and sealed web of felt impregnated with a bituminous saturant and squeezed by pressure mechanically applied to the surfaces on the opposite sides thereof and containing as squeezed less than 2% of voids and sealed on the opposite sides thereof in said deviated condition with a waterproofing material applied to said surfaces of said squeezed web without substantial absorption, or re-entry of air, which waterproofing material has a higher softening point than the softening point of said saturant and which waterproofing material is integrally bonded with said saturant and with the fibers of said web adjacent to and at said surfaces of said web and fills the surface interstices of said web to substantial depth, said web of felt as thus impregnated and sealed and including the body portion impregnated with the bituminous saturant and

the portions adjacent said surfaces sealed with said waterproofing material being so filled with said bituminous saturant and with said waterproofing material as to contain less than 2% of voids and being highly resistant to blistering.

4. As a roofing material, a filled and sealed web of felt, said felt web being impregnated with bituminous saturant and squeezed to a substantially deviated condition by pressure mechanically applied to opposite sides thereof and said felt web being sealed in said deviated condition on the opposite sides thereof by bituminous sealing material applied to the surfaces of said web on said opposite sides thereof, which bituminous sealing material has a higher softening point than the softening point of said saturant and both penetrates the said felt and fills the surface interstices of said felt at and adjacent the said surfaces of said felt to substantial depth, said filled and sealed web containing as a whole no more than 0.5% of voids and being highly resistant to blistering.

HAROLD W. GREIDER.  
GEORGE ARTHUR FASOLD.